

# United States Patent [19]

[ 19 ]

Konev et al.

[11] 3,759,386

[45] Sept. 18, 1973

[54] METHODS FOR FLOTATION OF ORES

[76] Inventors: **Vyacheslav Alexandrovich Konev**,  
Gavanskaya ulitsa, 16, kv. 6;  
**Vladimir Ilich Ryaboi**, Kostromskoi  
prospekt, 39, kv. 2, both of  
Leningrad, U.S.S.R.

[22] Filed: Oct. 23, 1970

[21] Appl. No.: 83,647

**[30] Foreign Application Priority Data**

Oct. 23, 1969 U.S.S.R. .... 1370210

[52] U.S. Cl. .... 209/167  
[51] Int. Cl. .... B03d 1/02  
[58] Field of Search .... 209/166, 167

**[56] References Cited**

## UNITED STATES PATENTS

|           |         |               |         |
|-----------|---------|---------------|---------|
| 1,988,052 | 1/1935  | Schafer ..... | 209/166 |
| 2,492,936 | 12/1949 | Nokes .....   | 209/167 |
| 2,608,298 | 8/1952  | Arbiter ..... | 209/167 |
| 2,811,255 | 10/1957 | Nokes .....   | 209/167 |

## FOREIGN PATENTS OR APPLICATIONS

120,787 5/1958 U.S.S.R..... 209/166  
123,098 3/1958 U.S.S.R..... 209/166

#### OTHER PUBLICATIONS

Chem. Abst., 68, 1968, 116535 m, pg. 112.

Chem. Abst., 70, 1969, 59,801 k, pg. 139.

*Primary Examiner*—Frank W. Lutter

*Assistant Examiner—Robert Halper*

Attorney—Holman & Stern

[57] ABSTRACT

A method for flotation of non-ferrous ores which includes flotation of said ore with separation of a bulk concentrate and tailings. The bulk concentrate produced is then conditioned with a desorbate agent containing a substance with the general chemical formula



wherein X is the second radical.



or sulphur. After this the bulk concentrate conditioned with said agent is subjected to selective flotation. Prior to selective floatation it is expedient to add a reagent reducing the pH of the pulp.

**2 Claims, No Drawings**

## METHODS FOR FLOTATION OF ORES

This invention relates to the area of mineral processing, and more particularly, to methods for flotation of ores containing non-ferrous metals such as zinc, lead, copper and molybdenum.

Well known are methods for flotation of polymetallic and lead-zinc ores, including selective flotation of lead- and copper minerals into a concentrate with subsequent recovery of zinc minerals.

For this purpose all the ore being processed is to be subjected to fine grinding for liberation of minerals, and for separation of useful constituents from each other and from the gangue. The process of grinding is power consuming, furthermore wear of grinding media and equipment is considerable. All the ore flow treated is repeatedly subjected to flotation with the use of different agents for consecutive separation of useful constituents from the ore.

It is preferable first to separate all the sulphides containing useful metals from the gangue amounting to 90 percent of the ore weight and to exclude this component from further treatment.

Also, the advantage of preliminary bulk flotation of sulphides is obvious too, as for their separation from the gangue by flotation, only coarse grinding is sufficient.

However, the sulphides first separated simultaneously are more difficult to separate later on from each other, because they are covered with a collector agent layer, feature similar flotation properties and yield only partially to the action of depressing agents.

To facilitate the action of depressing agents upon the sulfides, they are floated into a bulk concentrate at a collector agent quantity less than optimal, but this floating leads to their losses into tailings.

It has been attempted to separate a bulk concentrate from the ore to condition it with sodium sulphide and to subject it to treatment in classifiers and thickeners for washing off the reagents. However, this method too requires a considerable consumption of reagents (sodium sulphide) while classifiers and thickeners require large operation areas, and, consequently involve considerable capital investments and operational costs. In addition non-ferrous metals are lost in the thickener overflow.

The object of the present invention is to eliminate the difficulties previously mentioned.

The principal object of this invention is the provision of a method for flotation of non-ferrous ores which will ensure the improvement in grade and quantity of flotation concentrates produced, and will be more economically practical and easy to realize.

Said principal and other objects of the invention will be achieved through the realization of the herein-proposed method for flotation of non-ferrous ores, including: flotation of said ore with the separating of the bulk concentrate and tailings, conditioning of the bulk concentrate, obtained according to the invention, with an agent-desorbate containing a substance with the general chemical formula



where X is sulphur or the second radical



, and selective flotation with known reagents, of the bulk concentrate conditioned with the agent-desorbate.

Such a method ensures the production of more pure concentrates of metals, as well as their more complete recovery. In addition no washing of the bulk concentrates is required for the removal of agents, and thus losses of useful constituents in the overflow are avoided, no extra equipment such as classifiers and thickeners is needed, and thus the operation is not cumbersome. In consequence, capital investments and operational expenses are reduced.

While carrying out the method, it is expedient to use as an agent-desorbate the product of reaction of sodium sulphide with phosphorus trichloride.

Such an agent ensures the required rate of the collector desorption from the minerals to be separated at a relatively small consumption of the desorbate agent.

It is very expedient, prior to selective flotation to add to the bulk concentrate conditioned with the desorbate agent a reagent reducing the pH of the pulp.

This will ensure a more complete desorption of the collector from the surface of the minerals depressed.

Sulphuric acid may be used as an agent reducing the pH of the pulp. This will allow a reduction in the cost of such agents.

In order to explain the invention, an example of the proposed method of realization is described below.

An ore containing lead, zinc and pyrite is subjected to bulk flotation with potassium butyl xanthogenate as a collector. Thus a bulk concentrate and final tailings are obtained. This bulk concentrate is conditioned for 5 minutes with a solution of a desorbate agent containing a substance with the chemical formula



where X is the second radical of



The desorbate agent is produced as a result of the interaction of technical sodium sulphide with phosphorus trichloride. The desorbate agent consumption amounts to 400-500 g per ton of bulk concentrate (50 g/t of ore in terms of  $Na_4P_2S_6$ ). Following this, sulphuric acid as an agent for reducing the pH of the pulp pH is added to the bulk concentrate and conditioned for 10 minutes. The sulphuric acid consumption amounts to 1500-2000 g per ton of bulk concentrate (150-200 g/t of ore). Subsequently depressors used usually for sphalerite and pyrite are added to the pulp: sodium cyanide — 1000 g per ton of bulk concentrate (100 g/t of ore) and zinc sulphate — 3500 g per ton of bulk concentrate (350 g/t of ore) as well as sodium hydroxide as a pulp alkalinity modifier down to pH = 9.5. For 10 minutes the bulk concentrate is conditioned with these agents; then potassium butyl xanthogenate

— 40 g per ton of bulk concentrate (4 g/t of ore) and a frother are added till normal froth is formed, following which lead flotation is carried out.

While effectuating the procedure the use of the desorbate agent, more oxidation-resistant than sodium sulphide, allows the taking advantage of the selectivity of the very process of the collector desorption from the surface of sulphides, thus improving the technological data of the subsequent separation of useful minerals.

Said agent is a stronger desorbate of xanthogenate from the surface of sulphide minerals than sodium sulphide, thus allowing a considerable reduction in the consumption of the agent-desorbate.

The elimination of the operation of washing off the agents avoids the considerable capital investments and operational expenses required for such washing, and excludes metal losses in the overflow of the washing thickeners. Furthermore, it thus becomes possible to regulate and maintain at an optimum degree the collector removal from the surface of minerals to be separated.

Tests have shown that the results of the use of the present method for the flotation of non-ferrous ores can be considerably better than those obtained when using other methods. These results are shown in Tables 1 and 2; they refer to the separation of galena from sphalerite and pyrite carried out both in conformity with the present method, and with the known method, based on the desorption of the collector by sodium sulphide (Na<sub>2</sub>S consumption being 7000 g per ton of bulk concentrate) followed by washing off the agents (the washing off rate being 1:6).

TABLE I

Comparison of bulk concentrate separation results after the removal of the collector in conformity with the present and the known methods.

| Methods | Flotation product | Weight, percent | Content, percent |       | Recovery, percent |        |
|---------|-------------------|-----------------|------------------|-------|-------------------|--------|
|         |                   |                 | Lead             | Zinc  | Lead              | Zinc   |
| Known   | Lead concentrate  | 22.96           | 53.19            | 5.33  | 95.00             | 9.20   |
|         | Lead flotation    |                 |                  |       |                   |        |
|         | Tailings          | 77.04           | 0.84             | 16.23 | 5.00              | 90.80  |
| Present | Bulk concentrate  | 100.00          | 12.85            | 13.77 | 100.00            | 100.00 |
|         | Lead concentrate  | 17.40           | 59.51            | 5.48  | 95.70             | 7.45   |
|         | Lead flotation    |                 |                  |       |                   |        |
|         | Tailings          | 82.60           | 0.60             | 14.34 | 4.30              | 92.55  |
|         | Bulk concentrate  | 100.00          | 10.81            | 12.75 | 100.00            | 100.00 |

The data of Table I show that, where the present method was used, the results obtained were better than those obtained with the known method. Thus lead content in the lead concentrate was 6.32 percent higher and lead recovery into lead concentrate 0.7 percent higher, while zinc losses in the lead concentrate were 1.75 percent lower.

TABLE 2  
EXPENDITURE FOR AGENTS

| Methods | Agent | Agent consumption, g per ton of bulk concentrate | Cost per ton of agent | Expenses for each 1000 t of initial bulk concentrate, Rubles |
|---------|-------|--------------------------------------------------|-----------------------|--------------------------------------------------------------|
|         |       |                                                  |                       |                                                              |

The data in Table 2 show that the expenses for agents for the present method are 4.5 times lower than for the known method.

We claim:

1. A method for flotation of sulfide minerals which comprises: subjecting an ore to flotation with a collector reagent to separate a bulk sulfide concentrate and tailings, conditioning the bulk concentrate with a desorbate agent for said collector containing an inorganic hexathiohypophosphate compound, extracting the liquid phase of the conditioned bulk concentrate, diluting the thickened product with fresh water, and subjecting the obtained ready bulk concentrate to selective flotation of a sulfide mineral.

2. The method as claimed in claim 1, wherein said desorbate agent is the product obtained by the reaction of sodium sulfide with phosphorus trichloride.

\* \* \* \* \*